

## UNITED STATES PATENT OFFICE

BRUNO WENDT, OF DESSAU IN ANHALT, GERMANY, ASSIGNOR TO AGFA ANSCO CORPORATION, OF BINGHAMTON, NEW YORK, A CORPORATION OF NEW YORK

DESENSITIZER AND PROCESS OF DESENSITIZING LIGHT-SENSITIVE PHOTOGRAPHIC MATERIALS

No Drawing. Application filed December 28, 1928, Serial No. 329,070, and in Germany February 3, 1928.

The present invention relates to new desensitizing compounds for light sensitive photographic materials, more particularly it relates to the employment of polynuclear 5 quinones as desensitizers for silver halid emulsions.

These polynuclear quinones, especially anthraquinones and phenanthraquinones, have a powerful desensitizing effect and are 10 more powerful than the quinones of the benzene series. They are particularly applicable for desensitizing panchromatic emulsions.

In the groups of anthraquinones and phenanthraquinones are substances which are 15 active desensitizers and are at the same time not liable to color the photographic layer, though, of course, there are also bodies having 20 the properties of dyestuffs and the latter can be used in particular cases where coloration of the photographic layer is not objectionable.

Since the desensitizer must be used in 25 aqueous solution the anthraquinone or phenanthraquinone derivative selected should be soluble in water; for example it may be the sodium salt of the sulfonic acid.

The desensitizer may be used in a preliminary 30 bath or may be added to the developer solution. In the latter case very small proportions added will suffice for a considerable desensitizing so that the developer solution is not injuriously affected.

The following examples illustrate the invention:—

*Example 1.*—An exposed panchromatic plate or film is immersed for 2 minutes in the dark in a solution of sodium 1-nitro-40 anthraquinone-2-carboxylate (1:400). It may then be developed in red light.

*Example 2.*—A solution of alizarine direct blue B (Schultz, Farbstofftabellen, 5th edition, No. 851) of 0.1 per cent strength, may be 45 used in the manner described in Example 1.

*Example 3.*—To a suitable developer sodium anthraquinone-2-sulfonate is added so as to make its concentration in the solution 1:3000. The photographic film is immersed 50 in this developer for 2 minutes in the dark

and can then be further developed in red light.

I claim:

1. A process which comprises desensitizing 55 light sensitive photographic materials by treating them with an aqueous solution of a polynuclear quinone derivative.

2. A process which comprises desensitizing 60 light sensitive photographic materials by treating them with an aqueous solution of a polynuclear quinone containing a salt forming group.

3. A process which comprises desensitizing 65 light sensitive photographic materials by treating them with an aqueous solution of a salt of an acid derived from a polynuclear quinone.

4. A process which comprises desensitizing 70 light sensitive photographic materials by treating them with an aqueous solution of a salt of an acid derived from a polynuclear quinone containing at least one nitro-group.

5. A process which comprises desensitizing 75 light sensitive photographic materials by treating them with an aqueous solution of a salt of a sulfonic acid derived from a polynuclear quinone containing at least one nitro-group.

6. A process which comprises desensitizing 80 light sensitive photographic materials by treating them with an aqueous solution of a quinone derivative of the anthracene series.

7. A process which comprises desensitizing 85 light sensitive photographic materials by treating them with an aqueous solution of a quinone derivative of the anthracene series containing a salt forming group.

8. A process which comprises desensitizing 90 light sensitive photographic materials by treating them with an aqueous solution of a salt of an acid derived from anthraquinone.

9. A process which comprises desensitizing 95 light sensitive photographic materials by treating them with an aqueous solution of a salt of a sulfonic acid of anthraquinone.

10. A process which comprises desensitizing 100 light sensitive photographic materials by treating them with an aqueous solution of a salt of a mono-sulfonic acid of anthraquinone.

11. A process which comprises desensitizing light sensitive photographic materials by treating them with an aqueous solution of a salt of the anthraquinone-2-sulfonic acid.
- 5 12. A process which comprises desensitizing light sensitive photographic materials by treating them with an aqueous solution of sodium anthraquinone-2-sulfonate.
- 10 13. As a desensitizer a polynuclear quinone derivative soluble in water.
14. As a desensitizer a polynuclear quinone containing a salt forming group.
15. As a desensitizer a salt of an acid derived from a polynuclear quinone.
16. As a desensitizer a salt of an acid derived from a polynuclear quinone containing at least one nitro-group.
17. As a desensitizer a salt of a sulfonic acid derived from a polynuclear quinone containing at least one nitro-group.
18. As a desensitizer a quinone derivative of the anthracene series.
19. As a desensitizer a quinone derivative of the anthracene series containing a salt forming group.
- 20 20. As a desensitizer a salt of an acid derived from anthraquinone.
21. As a desensitizer a salt of a sulfonic acid of anthraquinone.
- 30 22. As a desensitizer a salt of a mono-sulfonic acid of anthraquinone.
23. As a desensitizer a salt of the anthraquinone-2-sulfonic acid.
- 35 24. As a desensitizer sodium anthraquinone-2-sulfonate.

In testimony whereof, I affix my signature.  
BRUNO WENDT.

40

45

50

55

60

65